

## UNITED STATES PATENT OFFICE

2,386,206

## MINERAL OIL COMPOSITION

John J. Giannmaria and Orland M. Reiff, Woodbury, N. J., assignors to Socony-Vacuum Oil Company, Incorporated, a corporation of New York

No Drawing. Application May 27, 1943,  
Serial No. 488,742

15 Claims. (Cl. 252—32.7)

This invention has to do in a general way with mineral oil compositions and is more particularly related to compositions comprised of mineral oil and a minor proportion of an added ingredient which will improve the oil in one or more important respects.

It is well known to those familiar with the art that mineral oil fractions refined for their various uses are in and of themselves usually deficient in one or more respects, so that their practical utility is limited even in the particular field for which they have been refined. For example, mineral oil fractions refined for use as lubricants have a tendency to oxidize under conditions of use with the formation of sludge or acidic oxidation products; also the lighter fractions such as gasoline and kerosene tend to oxidize with the formation of color bodies, gum, etc. In order to prevent or retard the formation of these products and thereby extend the useful life of the oil fraction, it is common practice to blend with such oil fractions an additive ingredient which will have the effect of inhibiting oxidation, such ingredients being generally known to the trade as oxidation inhibitors or sludge inhibitors, gum inhibitors, etc.

It is also the practice to add other ingredients to mineral oil fractions for the purpose of improving "oiliness" characteristics and the wear-reducing action of such mineral oils when they are used as lubricants, particularly when the oils are used for the purpose of lubricating metal surfaces which are engaged under extremely high pressures and at high rubbing speeds.

Other ingredients have been developed for the purpose of depressing the pour point of mineral oil fractions which have been refined for use as lubricants, such refinement leaving a certain amount of wax in the oil, which, without the added ingredient, would tend to crystallize at temperatures which would render the oil impracticable for use under low temperature conditions. Additive agents have also been developed for improving the viscosity index of lubricating oil fractions. In the case of internal combustion engines, particularly those operating with high cylinder pressures, there is a decided tendency for the ordinary lubricating oil fraction to form, under such conditions of use, carbonaceous deposits which cause the piston rings to become stuck in their slots and which fill the slots in the oil ring or rings, thus materially reducing the efficiency of the engine. Ingredients have, therefore, been developed which, when added to the oil, will reduce the natural tendency of the oil

to form deposits which interfere with the function of the piston rings.

Aside from the corrosive action which attends the formation of acidic products of oxidation in mineral oil fractions of the lubricant range, it has been discovered that certain types of recently developed hard metal alloy bearing metals, such as typified by cadmium-silver alloy bearings, are attacked by ingredients in certain types of oils, particularly oils of high viscosity index obtained by various methods of solvent-refining. This corrosive action on alloys of the aforesaid type has led to the development of corrosion inhibitors which may be used in solvent-refined oils to protect such bearing metals against this corrosive action.

In the lighter mineral oil fractions, such as those used for fuel purposes, particularly in internal combustion engines, it has been found that the combustion characteristics of the fuel may be controlled and improved by adding minor portions of various improving agents thereto.

The various ingredients which have been developed for use in mineral oil fractions to improve such fractions in the various respects enumerated above are largely specific to their particular applications, and it has, therefore, been the practise to add a separate ingredient for each of the improvements which is to be effected.

We have discovered that mineral oil fractions such as those referred to above can be improved in several of the various properties enumerated above by the incorporation therein of a small quantity of a multi-functional compound or reaction product selected from a new and novel class of phosphorus- and sulfur-containing compounds or reaction products. More specifically, we have found that the compounds or reaction products obtained by the reaction of substantially two mols of alkyl-substituted hydroxyaromatic carboxylic acids and one mol of phosphorus pentasulfide, and the metal salts thereof, improve such oil fractions in more than one of said properties. Particularly preferred, however, of these multifunctional oil addition agents are those compounds or reaction products of the aforesaid class which contain one or more oil-solubilizing "heavy" alkyl groups, that is, aliphatic hydrocarbon groups of relatively high molecular weight preferably containing not less than 20 carbon atoms, in the aromatic nucleus or aromatic nuclei.

The multifunctional oil addition agents of this invention are referred to as compounds and as reaction products inasmuch as both definite com-

pounds and products of indefinite chemical structure are obtained by reaction of substantially two mols of an alkyl-substituted hydroxyaromatic carboxylic acid and one mol of phosphorus pentasulfide. On the basis of chemical analyses of the phosphorus- and sulfur-containing products of this reaction, the principal product appears to be a combined thiophosphate esteraryl thiolic acid,



and the most probable reaction mechanism is



wherein T is an aromatic nucleus, either mono- or polycyclic, such as phenyl, naphthyl, anthracyl, etc.; R is an oil solubilizing aliphatic hydrocarbon radical or group containing at least about 18 carbon atoms, and is preferably a high molecular weight derivative or a heavy alkyl group, and n is a small whole number, preferably 1 to 4.

As aforesaid, also contemplated herein are the metal salts of the phosphorus- and sulfur-containing compounds and reaction products obtained by reaction of two mols of the aforesaid carboxylic acids and one mol of  $\text{P}_2\text{S}_5$ , wherein a metal (M) replaces the hydrogen of the thiolic acid group, —COSH. Thus, the metal salts of mixed thiophosphate ester-aryl thiolic acids may be represented by the following formula,



wherein M represents at least one metal equivalent, and R and n are as defined above. As contemplated herein the metal salts represented by Formula III are inclusive of both the neutral metal salts, wherein M will represent a metal atom such as —Na, —Ba—, etc., and the basic metal salts of said acids. In the latter salts, the symbol M, which represents at least one metal equivalent, is broadly construed to represent a basic metal grouping which is defined herein as a polyvalent metal atom having at least one valence satisfied by a hydroxide group or an alcoholate group, and having at least one valence satisfied as shown in Formula III.

The metal substituent in the thiolic acid group of the oil-improving agents described herein may be broadly classified as follows: the alkali metals, lithium, sodium, potassium, rubidium and caesium; the alkaline earth group, beryllium, magnesium, calcium, strontium and barium; the metals zinc, cadmium and mercury, scandium, yttrium, lanthanum, aluminium, gallium, indium, thallium, titanium, zirconium, cerium, thorium; germanium, tin and lead; vanadium, columbium and tantalum; arsenic, antimony and bismuth; chromium, molybdenum, tungsten and uranium; rhenium, manganese, iron, cobalt and nickel; ruthenium, rhodium and palladium; osmium, iridium and platinum.

Some of the rare earth metals are given in the above group of metals; other rare earths suitable for the formation of combined thiophosphate ester-aryl thiolic acid salts are those now

commercially available as the cerium and yttrium groups, namely, a mixture of praseodymium, neodymium, samarium, europium, gadolinium, terbium, dysprosium, holmium, erbium, thalium, and lutecium.

Particularly preferred metals for the salts contemplated herein are barium, tin and cobalt.

The combined thiophosphate ester-thiolic acids and salts described above may also be characterized by another substituent group, or groups, on the aromatic nucleus. That is, in addition to the alkyl, thiophosphate ester (—OPOS) and thiolic acid (—COSH, or metal thiolate —COSM) groups on the aromatic nucleus, other nuclear hydrogen atoms may be replaced by a monovalent substituent, or substituents, selected from the group consisting of hydroxyl, metaloxy, alkoxy, aroxy, ester, aralkyl, alkaryl, aryl, alkyl, (such as short-chain groups, methyl, ethyl, etc., in addition to the preferred long-chain R groups), halogen, nitro and nitroso; all of these substituents will be hereinafter referred to as Y substituents. Still other Y substituents which may be present are those having a multiple valence and these include the mono- and poly-sulfide-selenide and -telluride groups; of these groups, the disulfide group is particularly preferred. Thus the compounds containing a Y substituent, or substituents, will be represented by the formula



wherein Y is nuclear hydrogen or a group such as defined above; r is the numeral 0 or a small whole number, from 1 to 3, corresponding to the valences

40 on the nucleus T not satisfied by R, —OPOS and —COOX groups; X is hydrogen or at least one metal equivalent and the symbols T, R and n are as defined hereinbefore.

It will be apparent that those compounds contemplated herein which contain a Y substituent having a multiple valence, such for example as a disulfide group, will be characterized by more than one combined thiophosphate ester-thiolic acid (or metal thiolate) aryl nucleus, and that such compounds will be represented by the following general formula



wherein  $\Sigma$  is a substituent having a multiple valence and is selected from the group consisting of mono- and poly-sulfide, -selenide and -telluride groups; m is 0 or a small whole number, preferably from 1 to 2; and all other symbols are as defined hereinabove.

From the foregoing, therefore, it will be apparent that the symbol Y is of such scope as to include the following groups: nuclear hydrogen and the aforesaid monovalent substituents and multi-valent substituents and the group



in which  $\Sigma$  is representative of the aforesaid multivalent substituents and the symbols  $m$ ,  $T$ ,  $X$ ,  $R$  and  $n$  are as defined hereinabove.

As indicated above, the particularly preferred type of compounds or reaction products contemplated by the present invention are those represented by Formulae I, III and IV(a) and (b), in which the group represented by  $R$  is an aliphatic hydrocarbon radical of relatively high molecular weight, preferably containing not less than 20 carbon atoms. In the foregoing formulae (I, III and IV(a) and (b)) it will be observed that the aliphatic or alkyl substituent in the aryl nucleus is a monovalent aliphatic hydrocarbon group, but, as will appear from the hereinafter described synthesis of our preferred type of oil-improving agent, part or all of the aliphatic hydrocarbon material may be comprised of polyvalent aliphatic hydrocarbon radicals or groups in which the several valances are attached to separate aromatic nuclear groups. Compounds of this type are included under the following general formula representation



in which  $R$ ,  $T$ ,  $X$ ,  $Y$ ,  $\Sigma$ ,  $r$  and  $m$  have the same significance indicated above;  $R^v$  represents at least one oil-solubilizing aliphatic or alkyl radical or group, such alkyl group or groups being attached by one valance only to at least one aromatic nucleus  $T$ ,  $v$  representing the valance of the aliphatic radical  $R^v$  which may be a small whole number from 1 to 4; and  $u$  represents a whole number from 1 to 4 and indicates the total number of groups



present in the molecules represented by the formulae and which are attached to the aliphatic groups or groups represented by  $R^v$  through the valence or valences  $v$ :

In the foregoing general formula representation V, it will be seen that the compounds represented thereby include those materials in which all of the nuclear aliphatic substituent is monovalent ( $v=1$  and  $u=1$ ) or in which all of the aliphatic substituent is polyvalent ( $v$  and  $u$  being equal to 2, 3, or 4) and since  $R^v$  is defined as being at least one aliphatic radical or group and may therefore include several such groups, it will be seen that the general formula V is inclusive of compounds having nuclear aliphatic groups or radicals of different valences (from 1 to 4) in the same molecule. Also it will be observed that since  $u$  may be any whole number from 1 to 4, the number of aromatic nuclei  $T$  in said molecules may likewise vary from 1 to 4. It will be seen, therefore, that the relationship between  $u$  and  $v$  in formula V, in its broadest aspect, is such that when  $u$  is equal to 1,  $v$  is equal to 1; and when  $u$  is greater than 1, the valence  $v$  of at least one of the  $R^v$ 's is equal to  $u$  (in order to tie the several nuclei or  $T$ 's together), the valence of any remaining  $R^v$ 's being any whole number equal to or less than  $u$ .

In the above general formula V, it will be understood that since the groups  $R^v$  are aliphatic hydrocarbon radicals of the chain type and are each attached by one valence only to each corresponding aromatic nucleus, the valence  $v$  of such radical or radicals is of necessity never greater than the number  $u$ , which indicates the

number of aromatic nuclei in the molecules and in formula V is always equal to 1 when  $u$  equals 1. Otherwise an  $R^v$  having a valence greater than the number ( $u$ ) of aromatic nuclei would either have some of its valences unsatisfied or else would form a condensed ring or rings of attachment at two or more points to one and the same aromatic nucleus. Such latter compounds, as readily indicated from the definition of  $R^v$ , are not considered as characterizing the product of the present invention although probably formed in some instances in minor amounts as unobjectionable by-products by certain of the methods of preparation herein disclosed.

The type of compounds coming under general formula V in which only the thiophosphate group ( $-OPOS$ ), one thiolic acid group or metal thiolate group ( $COSX$ ) and the oil-solubilizing group or groups ( $R^v$ ) are present on a monocyclic nucleus, are illustrated by the following formulae.

When  $v$  and  $u$  are each equal to 1 and one  $R$  group is present, the compounds are illustrated by



wherein the chain represents the oil-solubilizing alkyl substituent ( $R^v$ ), and the symbol  $X$  is as hereinabove defined.

Since group  $R$  has been defined as "at least one," it will be apparent that there may be more than one heavy alkyl substituent attached to the nucleus  $T$ , such a compound, where  $v$  and  $u$  are each 1 and in which there are two such monovalent  $R^v$  groups, may be represented by the following formula:



in which the chains and  $X$  are as defined above.

Compounds of the type satisfying the general formula V in which  $R^v$  is polyvalent and  $v$  and  $u$  are more than one and in which there is only one such polyvalent  $R^v$  group, may be illustrated by the following formula, in which the aryl nucleus  $T$  is again indicated for illustration as being monocyclic:



Under this same type of compound indicated by formula C there may be more than one polyvalent  $R^v$  group (represented by the chain), such a compound in which there are, for example, two

polyvalent R<sup>v</sup> groups being illustrated by the following formula:



Another possible molecular structure of compounds coming under formula V is that for a compound having more than one polyvalent  $Rv$  group, at least two of which have different valences, such as the following:



With regard to the possible number of  $R'$  groups which may make up a single molecule, this will vary to the extent to which it is desired to effect substitution of the nucleus with oil-solubilizing alkyl groups for obtaining the desired properties in the product and is, of course, limited by the number of valences on the aromatic nucleus which are available for substitution. As will be apparent to those skilled in the art, the maximum possible number of  $R'$  groups which can be attached to a single aromatic nucleus will vary as the nucleus is mono- or polycyclic and also as the nucleus is otherwise substituted. It will also be apparent that available valences on the nuclei may all be attached to polyvalent aliphatic substituents.

It will be understood that the oil-improving agents contemplated by this invention may be pure compounds satisfying the general Formula V (and the general formulae I, III, and IV(a) and (b)), described above with any one of the various mono- and polycyclic aromatic nuclei as T and the various substituents  $R^v$ , (OPOS), (COSX), (COOX) and Y described, the only requisite being that at least one nuclear hydrogen be substituted with a thiophosphate ester group, another nuclear hydrogen being substituted with a thiolic acid or metal thiolate group (COSX), and at least one nuclear hydrogen be substituted with an oil-solubilizing aliphatic radical or group ( $R^v$ ). However, in manufacturing the preferred oil-improving product of the present invention by the preferred method of procedure, as will appear hereinafter, the final oil-improving product obtained is normally or usually a mixture of different compounds corresponding to different values of  $v$  and  $u$  and to different numbers of aliphatic groups  $R^v$ . It is for this reason that we have designated the oil-improving agents contemplated herein as compounds and as reaction products, and intend the designation "reaction products" broadly to encompass the compounds obtained herein.

As has been emphasized hereinabove, it is important that the preferred oil-improving agents as represented by general formula V have nuclear

hydrogen in the aromatic nucleus T substituted with predominantly aliphatic material which

comprises a sufficient proportion of the composition as a whole to render the same miscible with the mineral oil fraction in which the improving agent is used under normal conditions of handling and use. It appears from the results of our

30 research that there is a critical range in the degree of alkylation of these improving agents below which the product or agent will not satisfy the requirements for oil-miscibility. Expressing this in another way, it appears that the hydroxyaromatic constituent ( $T-OH$ ), of the alkylated hydroxyaromatic carboxylic acid, from which the combined thiophosphate ester-thiolic acid is derived should not exceed a certain percentage of such alkylated hydroxyaromatic carboxylic acid.

35 40 This critical range of alkylation may be roughly expressed as the ratio by weight of  $(T(OH))_u$  to  $R^o (T(OH))_u$ .

The degree of alkylation and the critical range within which operative or preferred compounds can be obtained may also be expressed as the number of carbon atoms contained in the aliphatic substituents for each aryl nucleus in a given molecule or molecular structure.

given below in terms of molecular structure.

The critical range in the degree of alkylation, as defined above, of the aryl nucleus in the improving agents contemplated herein may vary with: (a) the mineral oil fraction in which the improving agent is to be used; (b) the aryl nucleus T (mono- or poly-cyclic); (c) the hydroxyl content of the aryl nucleus from which the thiophosphate ester substituent is derived (mono- or poly-hydric); (d) the character of aliphatic material comprising the (R<sup>v</sup>) substituent (straight or branched chain); (e) mono- or poly-substitution of the aryl nucleus; and (f) other substituents on the nucleus T, which may be of positive or negative or of neutral solubilizing activity.

In general it may be said that a polycyclic nucleus appears to require a higher degree of alkylation than a monocyclic nucleus; that a polyhydric nucleus requires a higher degree of alkylation than a monohydric nucleus; and that branched-chain aliphatic substituents have a somewhat greater solubilizing action than straight-chain solubilizing substituents.

In view of the foregoing variables it would be impracticable and probably misleading to attempt to give an expression and figure which would indicate accurately the proper ratio of hydroxy-  
aromatic constituent to the alkylated hydroxy-  
aromatic substituents.

aromatic constituent which would express a degree of aliphatic substitution satisfying all cases taking these variables into account. As a guide for preparing the improving agents of this invention, however, our research indicates that for a product having poor depressing and viscosity index (V. I.) improving properties in addition to other valuable properties the ratio, expressed as:



should not be greater than 0.20 when the weight of the hydroxy-aromatic component  $(T(OH))_v$  is expressed in terms of its chemically equivalent weight of phenol. It will be observed that the ratio as expressed by Formula VI above does not take into account any other substituent in the nucleus than the aliphatic substituent and the hydroxyl group (which appears as a thiophosphate ester group in the final product), but since the aliphatic substituent is primarily relied upon as the solubilizing medium in the combined thiophosphate ester-thiolic acids (and salts thereof) derived from the aforesaid hydroxyaromatic acids, it is believed that the foregoing expression and limits will serve as a working guide for the preparation of oil-soluble materials and particularly of the preferred multifunctional reaction products and compounds contemplated herein.

The ratio of 20 per cent, which we may term the "phenolic ratio," represents what we consider a maximum figure for the preferred products of this invention, and in general it will be found that this figure will be lower. The actual ratio, of course, depends upon the variable factors enumerated above. For example, as will appear hereinafter, an oil-soluble combined thiophosphate ester-thiolic acid (and the metal salts thereof) of the multifunctional type in which the aliphatic substituent is derived from petroleum wax, a predominantly straight-chain aliphatic hydrocarbon of at least 20 carbon atoms, and in which the aromatic nucleus was derived from phenol otherwise unsubstituted should have a phenolic ratio, as expressed above, not substantially greater than about 16 per cent.

The degree of alkylation for these preferred multifunctional oil-improving agents may also be expressed by the number of carbon atoms contained in the aliphatic substituent for a given hydroxy-aromatic nucleus  $T-OH$ . As a general guide in this connection it may be said that the substituents represented by  $R^v$  in the above general Formula V should, for these preferred compounds or reaction products, contain at least twenty carbon atoms for each aromatic nucleus.

The alkylated hydroxyaromatic carboxylic acids which are reacted herein with  $P_2S_5$  in the molar proportion of 2:1 are preferably obtained by the procedures described in Patent 2,197,837, issued for one of the present inventors, O. M. Reiff. As described therein, numerous hydroxyaromatic compounds may be used as the starting materials and alkylated, and thereafter carboxylated. Examples of the hydroxyaromatic compounds which may be used as starting materials for the alkylation reaction are: phenol, resorcinol, hydroquinone, catechol, cresol, xylanol, hydroxydiphenyl, benzylphenol, phenyl-ethyl-phenol phenol resins, methyl hydroxydiphenyl, guaiacol, alpha- and beta-naphthol, tolyl naphthol, xylanol naphthol, benzyl naphthol, anthranol, phenyl methyl naphthol, phenanthrol, anisole, beta

naphthyl methyl ether, chlorphenol and the like. Preference is given to the monohydroxy phenols otherwise unsubstituted, particular preference being given to phenol and alpha- and beta-naphthol.

As indicated in said patent (2,197,837), the alkylation of the hydroxyaromatic compound may be accomplished in various ways, such as by Friedel-Crafts synthesis using a halogenated aliphatic hydrocarbon; by reaction with unsaturated high molecular weight aliphatic compounds or higher alcohols in the presence of a suitable catalyst such as sulfuric acid, etc. The Friedel-Crafts type of alkylation reaction, however, is particularly adapted to the preparation of the alkylated hydroxyaromatic compounds from which the corresponding acids are obtained because the Friedel-Crafts synthesis affords a convenient means of controlling the degree of alkylation and obtaining the desired phenolic ratio.

In this latter type of synthesis an appropriate mono- or poly-chlorine-substituted aliphatic compound or material is reacted with the desired hydroxyaromatic compound in the presence of a Friedel-Crafts catalyst such as a catalytic amount of aluminum chloride. Pure or substantially pure chlorinated aliphatic compounds may be used. As will be readily understood by those skilled in the art, it is usually difficult to prepare or obtain high molecular weight aliphatic hydrocarbons in a pure or substantially pure state and correspondingly difficult to prepare the chlorine- or other halogen-substituted products in a pure or substantially pure state. It is preferred, therefore, to employ a mixture of such halogenated hydrocarbons, such as halogenated petroleum fractions, as the starting material. In general it may be said that the high molecular weight aliphatic hydrocarbons contemplated as preferred sources for the alkyl substituent  $R^v$  in Formula V for obtaining the multifunctional phosphorus- and sulfur-containing oil addition agents of this invention, may be pure or mixed compounds typified by those which characterize the heavy products of petroleum, such as heavy petroleum oils, crystalline petroleum wax, etc., or other compounds or materials which will result in relatively long hydrocarbon chain substituents. Special preference is given to petroleum wax having a melting point not substantially less than about 120° F. and having a molecular weight of about 300 and at least twenty carbon atoms in the characterizing molecules.

Since the product of a Friedel-Crafts reaction between a chlorinated aliphatic material of the type referred to above and a hydroxyaromatic compound will be a mixture of different values of  $v$  and  $u$  in the formula  $R^v(T(OH))_u$  shown above in describing the "phenolic ratio," and the final thiophosphate ester-thiolic acids (and salts thereof) derived therefrom will likewise be a mixture of compounds corresponding to different values of  $v$  and  $u$  in general formula V, it will be understood that the specific values for  $v$  and  $u$  in the above formula as well as the general formula V relate to the different specific compounds present in such a mixture which characterize it as a reaction product of this invention.

Following alkylation of the desired hydroxyaromatic compound, the alkylated reaction product thus obtained is carboxylated according to the procedures outlined in Patent 2,197,837. As indicated therein, one suitable procedure involves first forming an alkyl-substituted metal hydroxylate from an alkyl-substituted hydroxy-aromatic

compound and a metal such as an alkali or alkaline earth, and then carboxylating the hydroxylate (obtained in the preceding operation) with carbon dioxide gas to form the alkylated hydroxyaromatic carboxylic acid. The latter product is available for reaction with  $P_2S_5$  to provide the multifunctional oil-improving agents of this invention. Typical alkylated hydroxyaromatic carboxylic acids which may be reacted with  $P_2S_5$  as hereinafter described, include the carboxylic acids of the representative hydroxyaromatic compounds enumerated above. Preferred herein are alkylated phenol and naphthol carboxylic acids.

In the event that an aliphatic material such as petroleum wax described above is used as the alkyl substituent on the hydroxyaromatic compound and corresponding hydroxyaromatic carboxylic acid derived therefrom, and is reacted in the form of halogenated wax containing, for example, three atomic proportions of chlorine and 14 per cent chlorine, with one mol of said hydroxyaromatic compound, the alkylated hydroxyaromatic compound and the alkylated hydroxyaromatic carboxylic acid will be, for convenience, designated hereinafter as "wax-hydroxyaromatic compound (3-14)" and "wax-hydroxyaromatic carboxylic acid (3-14)," respectively. Parenthetical expression of the type (A-B) may be used hereinafter in connection with such compounds to designate (A) the number of atomic proportions in the chloraliphatic material which was reacted with one mol of hydroxyaromatic compound in the Friedel-Crafts reaction and (B) the chlorine content of the chloraliphatic material. In the above illustrations A=3 and B=14.

This same designation will also apply to the alkylated thiophosphate ester-thiolic acids, and their metal salts, derived from these alkylated compounds.

The multifunctional phosphorus- and sulfur-containing oil improving agents of this invention are obtained by reaction of substantially two mols of an alkylated hydroxyaromatic carboxylic acid of the type described above and one mol of  $P_2S_5$ . They may also be obtained by reaction of the alkali or alkaline earth metal salts of the aforesaid alkylated hydroxyaromatic carboxylic acid and  $P_2S_5$  in the same molar ratio, but the preferred procedure is that one in which the metal-free carboxylic acid reactant is used. The procedures outlined above will be illustrated by the following examples, wherein reaction products typical of the aforesaid reaction products are prepared.

#### REACTION OF ALKYL-SUBSTITUTED HYDROXYAROMATIC CARBOXYLIC ACIDS AND $P_2S_5$

##### EXAMPLE 1

*Reaction of wax-substituted phenol carboxylic acid and  $P_2S_5$*

(a) Reaction mixture:

|                                                                                                          | Grams |
|----------------------------------------------------------------------------------------------------------|-------|
| Wax-phenol carboxylic acid (3-14) in solution in 300 grams of mineral oil (67 secs. S. U. V. at 120° F.) | 100   |
| $P_2S_5$                                                                                                 | 13.1  |
| Ethylene dichloride                                                                                      | 200   |

(b) Procedure:

The wax-phenol carboxylic acid in mineral oil blend, prepared according to the procedure in

Patent 2,197,837, is mixed with  $P_2S_5$ , the mol ratio of acid to  $P_2S_5$  being about 2:1, in a reaction vessel equipped with stirrer and reflux condenser. The mixture is diluted with  $\frac{1}{2}$  part of ethylene dichloride, 200 grams, and heated at the reflux temperature for about 10 hours to bring about reaction of said acid with  $P_2S_5$ . The mixture is then filtered and the ethylene dichloride solvent is distilled from the filtrate whereby the finished product, the combined thiophosphate ester-thiolic acid of wax-phenol carboxylic acid is obtained in mineral oil. Chemical analysis of the product indicates that the formula for such product is,



wherein  $R_n$  is wax.

##### EXAMPLE 2

*Reaction of wax-substituted phenol carboxylic acid disulfide and  $P_2S_5$*

(a) Reaction mixture:

|                                                                                                                    | Grams |
|--------------------------------------------------------------------------------------------------------------------|-------|
| Wax-phenol carboxylic acid disulfide (3-14) in solution in 300 grams of mineral oil (67 secs. S. U. V. at 310° F.) | 100   |
| $P_2S_5$                                                                                                           | 13.1  |
| Ethylene dichloride                                                                                                | 200   |

(b) Procedure:

The reaction of wax-phenol carboxylic acid disulfide, obtained as described in co-pending application of Serial No. 330,532, filed by O. M. Reiff on April 19, 1940, now issued as Patent No. 2,319,189 of May 11, 1943, was carried out according to the procedure given in Example 1, and here again the molar ratio of the acid disulfide to  $P_2S_5$  was about 2:1. The reaction product, in mineral oil blend, is believed to be the combined thiophosphate ester-thiolic acid of wax-phenol carboxylic acid disulfide and the formula for such product is believed to be,



wherein  $R_n$  is wax.

As aforesaid, the neutral and basic metal salts of the aforesaid reaction products are also contemplated by this invention. These metal-containing products are obtained by reaction of the combined thiophosphate ester-thiolic acids of the alkyl-substituted hydroxyaromatic carboxylic acids with alkali or alkaline earth metal alcoholates or hydroxides. In the use of the metal alcoholates, the thiophosphate ester-thiolic acid reaction product is diluted with one part of butanol, followed by adding the metal alcoholate, preferably as the metal butylate, heating the reaction mixture to the reflux temperature for one hour and then distilling off the alcohol—such as

butanol—to obtain the finished product, the corresponding metal salt. In the use of metal hydroxides, the combined thiophosphate ester-thiolic acid reaction product is diluted with  $\frac{1}{2}$  part of benzol, followed by adding the metal hydroxide. The reaction mixture is heated gently at the distillation temperature of benzol whereupon the water of reaction is removed. Any hydroxide residue is removed by filtering the reaction mixture and then distilling off the remaining benzol from the filtrate to obtain the finished product.

Metal salts of the phosphorus- and sulfur-containing reaction products described above, other than those of the alkali or alkaline earth metals, are formed by double decomposition of an alkali or alkaline earth metal salt with an alcohol solution of the chloride of the desired metal. The general procedure consists of dissolving the metal chloride in butanol and slowly adding the butanol solution thus obtained to the alkali (or alkaline earth) metal salt of the thiophosphate ester-thiolic acid reaction product. The mixture thus formed is heated at the reflux temperature for about 30 minutes and the alcohol solvent is then distilled off. The solvent-free mixture is then filtered through a suitable filter medium such as Hi-Flow to remove alkali (or alkaline earth) chloride formed as a by-product; the filtrate is the finished metal salt of said reaction product.

The alcoholate method of forming metal derivatives, as outlined above, is also applicable to metals other than the alkali or alkaline earth group. The desired metal alcoholates are formed by double decomposition of alkali alcoholate with an alcohol solution of the chloride of the desired metal. This mixture can then be reacted directly with the combined thiophosphate ester-thiolic acid reaction product described above to form the metal derivative. The alkali chloride formed as a by-product in preparing the alcoholate of the desired metal is filtered from the reaction product to give the finished material.

The metal salts contemplated herein are illustrated by the following examples.

### EXAMPLE 3

#### *Barium salt of the thiophosphate ester-thiolic acid of wax-phenol carboxylic acid (3-14)*

##### (a) Reaction mixture:

|                                                                                                                                              | Grams | 55 |
|----------------------------------------------------------------------------------------------------------------------------------------------|-------|----|
| Thiophosphate ester-thiolic acid of wax-phenol carboxylic acid (3-14) in solution in 300 grams of mineral oil (67 secs. S. U. V. at 210° F.) | 100   |    |
| Benzol                                                                                                                                       | 200   | 60 |
| Ba(OH) <sub>2</sub> ·8H <sub>2</sub> O                                                                                                       | 37    |    |

##### (b) Procedure:

The mineral oil blend containing the combined thiophosphate ester-thiolic acid of wax-phenol carboxylic acid (3-14), obtained in Example 1, was diluted with benzol and then treated with the barium hydroxide. The reaction mixture was then heated so that the benzol slowly distilled off carrying with it the water of reaction. Any barium hydroxide residue is removed by filtering the reaction mixture through Hi-Flow before distilling off the remaining benzol. The finished product, the combined thiophosphate ester-barium thiolate of wax-phenol carboxylic

acid (3-14), is approximately a 25% solution in mineral oil, and is characterized by the representation,

5



15

wherein Rn is wax.

### EXAMPLE 4

#### *Stannous salt of the thiophosphate ester-thiolic acid of wax-phenol carboxylic acid (3-14)*

##### (a) Reaction mixture:

Thiophosphate ester-thiolic acid of wax-phenol carboxylic acid (3-14) in solution in 300 grams of mineral oil (67 secs. S. U. V. at 210° F.)

25

grams 100

Butanol cc 200

Metallic sodium grams 6

Stannous chloride do 24.8

30

##### (b) Procedure:

The mineral oil blend containing the combined thiophosphate ester-thiolic acid of wax-phenol carboxylic acid (3-14), obtained in Example 1, is diluted with 100 cc. of butanol. Sodium, in the form of thin strips, is then added and the mixture is heated at the reflux temperature until all of the sodium has reacted. Stannous chloride in solution in butanol is then added and the reaction mixture heated at reflux for about 30 minutes. Butanol is distilled from the reaction mixture and the butanol-free mixture is then cooled, diluted with benzol and filtered. The filtrate is then distilled to remove benzol therefrom to obtain a mineral oil blend of the finished product, the combined thiophosphate ester-stannous thiolate of wax-phenol carboxylic acid (3-14) which is characterized by the representation,

35



wherein Rn is wax.

### EXAMPLE 5

#### *Barium salt of the thiophosphate ester-thiolic acid of wax-phenol carboxylic acid disulfide (3-14)*

##### (a) Reaction mixture:

|                                                                                                                                                        | Grams |
|--------------------------------------------------------------------------------------------------------------------------------------------------------|-------|
| Thiophosphate ester-thiolic acid of wax-phenol carboxylic acid disulfide (3-14) in solution in 300 grams of mineral oil (67 secs. S. U. V. at 210° F.) | 100   |
| Ba(OH) <sub>2</sub> ·8H <sub>2</sub> O                                                                                                                 | 37    |

##### (b) Procedure:

The method of preparation is the same as in

Example 4 and the finished product in this case is characterized by the representation



where  $R_n$  is wax..

REACTION OF ALKALINE EARTH METAL SALTS OF ALKYL-SUBSTITUTED HYDROXYAROMATIC CARBOXYLIC ACIDS AND  $P_2S_5$

EXAMPLE 6

Reaction of barium salt of diamyl-phenol carboxylic acid and  $P_2S_5$

(a) Reaction mixture:

|                                                                                                                    | Grams |
|--------------------------------------------------------------------------------------------------------------------|-------|
| Barium salt of diamyl phenol carboxylic acid in solution in 50 grams of mineral oil (67 secs. S. U. V. at 210° F.) | 50    |
| Benzol                                                                                                             | 50    |
| $P_2S_5$                                                                                                           | 12.8  |

(b) Procedure:

The barium salt of diamyl phenol carboxylic acid in mineral oil blend, obtained as described in a co-pending application Serial No. 452,054, filed July 23, 1943, in which one of the present inventors, O. M. Reiff, is a joint-inventor, is mixed with  $P_2S_5$  in a reaction vessel equipped with stirrer and reflux condenser. The mol ratio of the salt and  $P_2S_5$  is about 2:1. The mixture is diluted with benzol and heated at the reflux temperature for about 24 hours to bring about the reaction of said acid with  $P_2S_5$ . The benzol is then distilled from the reaction mixture and the temperature is raised thereafter to 125° C., and maintained for several hours to remove the  $H_2S$  formed in the reaction. The finished product, the combined thiophosphate ester-barium thiolate of diamyl phenol carboxylic acid, is thus obtained in a 1:1 oil blend, and is characterized by the representation



EXAMPLE 7

Reaction of barium salt of wax-phenol carboxylic acid disulfide (3-14) and  $P_2S_5$

(a) Reaction mixture:

|                                                                                                                                   | Grams |
|-----------------------------------------------------------------------------------------------------------------------------------|-------|
| Barium salt of wax-phenol carboxylic acid disulfide (3-14) in solution in 200 grams of mineral oil (67 secs. S. U. V. at 210° F.) | 100   |
| $P_2S_5$                                                                                                                          | 12.4  |

(b) Procedure:

The barium salt of wax-phenol carboxylic acid disulfide (3-14), in mineral oil blend, prepared as described in Patent 2,256,443, issued to one of

the present inventors, O. M. Reiff, was reacted with  $P_2S_5$ , in mol proportion of about 2:1 and the reaction product worked up as described in Example 6 above. The final reaction product is 5 presumably the same as the final reaction product obtained in Example 5, namely, the thiophosphate ester-barium thiolate of wax-phenol carboxylic acid disulfide; and, therefore, the formula given in Example 5 also represents the reaction product obtained in this example.

REACTION OF ALKALI METAL SALTS OF ALKYL-SUBSTITUTED HYDROXYAROMATIC CARBOXYLIC ACIDS AND  $P_2S_5$

EXAMPLE 8

Reaction of sodium carboxylate salt of diamyl-phenol carboxylic acid and  $P_2S_5$

|                                                                                                                     | Grams |
|---------------------------------------------------------------------------------------------------------------------|-------|
| Sodium carboxylate salt of diamyl-phenol carboxylic acid in 100 grams of mineral oil (67 secs. S. U. V. at 210° F.) | 50    |
| Benzol                                                                                                              | 100   |
| $P_2S_5$                                                                                                            | 18.5  |

(b) Procedure:

The procedure here is the same as in Example 6 and the final reaction product corresponds to the combined thiophosphate ester-sodium thiolate of diamyl-phenol carboxylic acid which may be represented by the formula



To demonstrate the effectiveness of these compounds or reaction products obtained by the reaction of substantially two mols of an alkyl-substituted hydroxyaromatic carboxylic acid and one mol of  $P_2S_5$ , and the metal salts thereof, in mineral oil compositions, we have conducted several comparative tests with representative mineral oils alone and with the same oils blended with typical compounds or reaction products of the class contemplated herein. These tests, which with their results are described below, show that mineral oil compositions containing these materials are improved as to pour point, viscosity index, and acidity during engine operation.

Pour point depression

The oil used in this test was a mineral lubricating oil fraction having a Saybolt Universal viscosity of 67 seconds at 210° F., and a pour point of +20° F. Using this oil, blends were prepared containing typical reaction products or compounds of this invention, namely, a combined thiophosphate ester-thiolic acid containing a "wax" substituent, and metal salts thereof, and the pour points of said blends determined. The results listed below in Table 1 demonstrate that the reaction products or compounds contemplated herein are extremely effective in lowering the pour point of the oil.

TABLE 1

| Improving agent                                                                          | A. S. T. M. pour point,<br>°F. |       |       |      |
|------------------------------------------------------------------------------------------|--------------------------------|-------|-------|------|
|                                                                                          | 0%                             | 1/16% | 1/16% | 1/4% |
| None                                                                                     | +20                            |       |       |      |
| Combined thiophosphate ester-thiolic acid of wax-phenol carboxylic acid (3-14)           | +20                            | 0     | -15   | -15  |
| Barium salt                                                                              | +20                            | +5    | -10   | -15  |
| Cobalt salt                                                                              | +20                            | 0     | -10   | -20  |
| Tin salt                                                                                 | +20                            | -5    | -15   | -20  |
| Calcium salt                                                                             | +20                            | 0     | -15   | -20  |
| Combined thiophosphate ester-thiolic acid of wax-phenol carboxylic acid disulfide (3-14) | +20                            | 0     | 0     | -20  |
| Barium salt                                                                              | +20                            | 0     | -10   | -20  |

**Viscosity index**

The results tabulated below in Table 2 demonstrate the comparative effectiveness of the reaction products or compounds contemplated herein as improvers of the viscosity index (V. I.) of motor oils. The oil used in these tests was a motor lubricating oil fraction having a kinematic viscosity of 30.17 and 4.80 at 100° F. and at 210° F., respectively, and a viscosity index of 79.8. It is apparent from these results that the oil improving agents of this invention effect an appreciable improvement in the viscosity index of the oil.

TABLE 2

| Improving agent blended with motor oil                                                   | Conc. by weight | Kinematic viscosity, centistokes, at— |         | V. I. |
|------------------------------------------------------------------------------------------|-----------------|---------------------------------------|---------|-------|
|                                                                                          |                 | 100° F.                               | 210° F. |       |
| None                                                                                     | 0               | 30.17                                 | 4.8     | 79.8  |
| Combined thiophosphate ester-thiolic acid of wax-phenol carboxylic acid (3-14)           | 1               | 33.10                                 | 5.10    | 85.0  |
| Barium salt                                                                              | 1               | 37.22                                 | 5.63    | 97.2  |
| Tin salt                                                                                 | 1               | 31.67                                 | 4.99    | 86.0  |
| Cobalt salt                                                                              | 1               | 32.02                                 | 5.00    | 84.2  |
| Calcium salt                                                                             | 1               | 31.78                                 | 4.97    | 83.3  |
| Combined thiophosphate ester-thiolic acid of wax-phenol carboxylic acid disulfide (3-14) | 1               | 31.98                                 | 4.98    | 82.6  |
| Barium salt                                                                              | 1               | 33.06                                 | 5.13    | 88.0  |

**Operation test**

We have also made comparative tests between an oil and oil blends containing representative improving agents of the type contemplated herein to determine the comparative behavior of the unblended oil and the improved oil under the actual operating conditions of an automotive engine. In order to determine the comparative effectiveness of an oil blend of the type contemplated herein, namely, one containing a metal salt prepared by using the aforesaid molar ratio of one mol of P<sub>2</sub>S<sub>5</sub> to two mols of an alkyl-substituted hydroxyaromatic carboxylic acid, and of an oil blend containing a metal salt prepared by using a different molar ratio, namely, one P<sub>2</sub>S<sub>5</sub> to four of said acid, similar comparative tests were carried out.

The tests were carried out in a single-cylinder Lauson engine operated continuously over a time interval of either 16, 24 or 36 hours with the cooling medium held at a temperature of about 212° F. and the oil temperature held at about 280° F. The engine was operated at a speed of about 1830 R. P. M. At the end of the test the oil was tested for acidity (N. N.) and viscosity.

The oil used in the test was a lubricating oil having a kinematic viscosity of 5.8 centistokes at 75

210° F. The results on the blank oil and the oil blends are listed in Table 3 below.

TABLE 3

| 5  | Improving agent blended with motor oil                                                        | Conc., percent | Hrs. run | N. N. | Kinematic vis. at 210° F. |
|----|-----------------------------------------------------------------------------------------------|----------------|----------|-------|---------------------------|
| 10 | None                                                                                          |                | 16       | 7.0   | 8.68                      |
|    | Combined thiophosphate ester-thiolic acid of wax-phenol carboxylic acid (3-14)                | 1              | 16       | 0.5   | 6.05                      |
|    | None                                                                                          |                | 24       | 4.9   | 7.09                      |
| 15 | Combined thiophosphate ester-barium thiolate of wax-phenol carboxylic acid (3-14) (Example 3) | 1              | 24       | 1.1   | 6.29                      |
|    | None                                                                                          |                | 16       | 7.0   | 8.68                      |
| 20 | Combined thiophosphate ester-barium thiolate of diethyl-phenol carboxylic acid (Example 6)    | 0.5            | 16       | 0.2   | 5.85                      |
|    | None                                                                                          |                | 24       | 6.1   | 8.20                      |
|    | Combined thiophosphate ester-thiolic acid of wax-phenol carboxylic acid disulfide (3-14)      | 1              | 24       | 0.9   | 6.07                      |
|    | None                                                                                          |                | 24       | 4.7   | 7.30                      |
| 25 | Combined thiophosphate ester-barium thiolate of wax-phenol carboxylic acid disulfide (3-14)   | 1              | 24       | 1.2   | 6.22                      |
|    | None                                                                                          |                | 36       | 6.8   | 9.82                      |
|    | Combined thiophosphate ester-barium thiolate of wax-phenol carboxylic acid (3-14) (1:4 ratio) | 0.25           | 36       | 4.8   | 7.74                      |
| 30 | Combined thiophosphate ester-barium thiolate of wax-phenol carboxylic acid (3-14) (1:2 ratio) | 0.25           | 36       | 7.1   | 9.00                      |
|    |                                                                                               |                |          |       | 6.46                      |

The data tabulated in Table 3 clearly show that the improving agents of this invention effect substantial improvement in mineral oil during actual operating conditions. Such data also show the superiority of these improving agents over related materials obtained by using a different molar ratio of reactants, namely, one mol of P<sub>2</sub>S<sub>5</sub> to four mols of an alkyl-substituted hydroxyaromatic carboxylic acid (or metal carboxylate thereof).

It will be apparent from the foregoing description that we have developed a new class of mineral oil compositions characterized by the presence of a minor proportion of a combined thiophosphate ester-thiolic acid of an alkylated hydroxyaromatic carboxylic acid, which is obtained by the reaction of substantially two mols of an alkylated hydroxyaromatic carboxylic acid and one mol of phosphorus pentasulfide, and the metal salts thereof. It is to be understood that the properties of the added agent may be varied by the degree of alkylation and the substituent groups on the aromatic nucleus in addition to the oil-solubilizing alkyl, thiophosphate ester, and thiolic acid (or metal thiolate) groups. It will be further understood that the improvement effected in the mineral oil composition may be varied by the amount of agent added. In general, it appears that the desired improvement can be effected by amounts varying from about  $\frac{1}{8}$  of one per cent to about 10 per cent, but the invention contemplates the use in amounts varying from  $\frac{1}{8}$  of one per cent to 2 per cent.

We claim:

1. An improved mineral oil composition comprising a mineral oil fraction having in admixture therewith a minor proportion, sufficient to stabilize said oil fraction against oxidation, of a compound characterized by the presence of an aromatic nucleus containing at least one oil-solubilizing alkyl group, a thiophosphate ester group (—OPOS), and a group selected from the group

consisting of a thiolic acid group and a metal thiolate group ( $-\text{COSX}$ ) wherein  $\text{X}$  is selected from the group consisting of hydrogen and at least one metal equivalent, said compound being obtained by the reaction of substantially two mols of a compound selected from the group consisting of an alkyl-substituted hydroxyaromatic carboxylic acid and an alkyl-substituted hydroxyaromatic metal carboxylate, the alkyl substituent being at least one oil-solubilizing alkyl group, and one mol of phosphorus pentasulfide.

2. An improved mineral oil composition comprising a mineral oil fraction having in admixture therewith a minor proportion, sufficient to stabilize said oil fraction against oxidation, of a compound characterized by the presence of an aromatic nucleus containing at least one oil-solubilizing alkyl group having at least twenty carbon atoms, a thiophosphate ester group ( $-\text{OPOS}$ ), and a group selected from the group consisting of a thiolic acid group and a metal thiolate group ( $-\text{COSX}$ ) wherein  $\text{X}$  is selected from the group consisting of hydrogen and at least one metal equivalent, said compound being obtained by the reaction of substantially two mols of a compound selected from the group consisting of an alkyl-substituted hydroxyaromatic carboxylic acid and an alkyl-substituted hydroxyaromatic metal carboxylate, the alkyl substituent being at least one oil-solubilizing alkyl group having at least twenty carbon atoms, and one mol of phosphorus pentasulfide.

3. An improved mineral oil composition comprising a mineral oil fraction having in admixture therewith a minor proportion, sufficient to stabilize said oil fraction against oxidation, of a compound characterized by the presence of an aromatic nucleus containing at least one oil-solubilizing alkyl group of the type which characterizes petroleum wax, a thiophosphate ester group ( $-\text{OPOS}$ ), and a group selected from the group consisting of a thiolic acid group and a metal thiolate group ( $-\text{COSX}$ ) wherein  $\text{X}$  is selected from the group consisting of hydrogen and at least one metal equivalent, said compound being obtained by the reaction of substantially two mols of a compound selected from the group consisting of an alkyl-substituted hydroxyaromatic carboxylic acid and an alkyl-substituted hydroxyaromatic metal carboxylate, the alkyl substituent being at least one oil-solubilizing alkyl group of the type which characterizes petroleum wax, and one mol of phosphorus pentasulfide.

4. An improved mineral oil composition comprising a mineral oil fraction having in admixture therewith a minor proportion, from about  $\frac{1}{8}$  per cent to about 10 per cent, of a compound characterized by the presence of an aromatic nucleus containing at least one oil-solubilizing alkyl group, a thiophosphate ester group ( $-\text{OPOS}$ ), and a group selected from the group consisting of a thiolic acid group and a metal thiolate group ( $-\text{COSX}$ ) wherein  $\text{X}$  is selected from the group consisting of hydrogen and at least one metal equivalent, said compound being obtained by the reaction of substantially two mols of a compound selected from the group consisting of an alkyl-substituted hydroxyaromatic carboxylic acid and an alkyl-substituted hydroxyaromatic metal carboxylate, the alkyl substituent being at least one oil-solubilizing alkyl group, and one mol of phosphorus pentasulfide.

5. An improved mineral oil composition comprising a mineral oil fraction having in admixture therewith a minor proportion, sufficient to stabilize

said oil fraction against oxidation, of a compound represented by the formula



wherein  $\text{T}$  is an aromatic nucleus;  $\text{X}$  is selected from the group consisting of hydrogen and at least one metal equivalent;  $\text{R}$  is at least one oil-solubilizing alkyl group;  $n$  is the number of said  $\text{R}$  groups and is a small whole number from 1 to 4; said compound being obtained by the reaction of one mol of phosphorus pentasulfide and substantially two mols of a compound selected from the group of compounds consisting of an alkyl-substituted hydroxyaromatic carboxylic acid and an alkyl-substituted hydroxyaromatic metal carboxylate, the alkyl substituent of said compound being at least one oil-solubilizing alkyl group ( $\text{R}$ ).

6. An improved mineral oil composition comprising a mineral oil fraction having in admixture therewith a minor proportion, sufficient to stabilize said oil fraction against oxidation, of a compound represented by the formula



wherein  $\text{R}^v$  represents at least one oil-solubilizing alkyl group, attached by one valence only to at least one aromatic nucleus  $\text{T}$ ;  $v$  represents the valence of said alkyl group  $\text{R}$  and is a small whole number from 1 to 4;  $\text{X}$  is selected from the group consisting of hydrogen and at least one metal equivalent;  $u$  is a small whole number from 1 to 4 and represents the total number of groups



attached to said alkyl group  $\text{R}^v$  through the valence  $v$ ; said compound being obtained by the reaction of one mol of phosphorus pentasulfide and substantially two mols of a compound selected from the group of compounds consisting of an alkyl-substituted hydroxyaromatic carboxylic acid and an alkyl-substituted hydroxyaromatic metal carboxylate, the alkyl substituent of said compound being at least one oil-solubilizing alkyl group.

7. An improved mineral oil composition comprising a mineral oil fraction having in admixture therewith a minor proportion, sufficient to stabilize said oil fraction against oxidation, of a compound represented by the formula



wherein  $\text{R}^v$  represents at least one oil-solubilizing alkyl group having at least twenty carbon atoms, attached by one valence only to at least one aromatic nucleus  $\text{T}$ ;  $v$  represents the valence of said alkyl group  $\text{R}$  and is a small whole number from 1 to 4;  $\text{X}$  is selected from the group consisting of hydrogen and at least one metal equivalent;  $u$  is a small whole number from 1 to 4 and represents the total number of groups



attached to said alkyl group  $\text{R}^v$  through the valence  $v$ ; said compound being obtained by the reaction of one mol of phosphorus pentasulfide and substantially two mols of a compound selected from the group of compounds consisting of an alkyl-substituted hydroxyaromatic carboxylic acid and an alkyl-substituted hydroxyaromatic metal carboxylate, the alkyl substituent of said compound being at least one oil-solubilizing alkyl group having at least twenty carbon atoms.

8. An improved mineral oil composition comprising a mineral oil fraction having in admixture therewith a minor proportion, sufficient to stabilize said oil fraction against oxidation, of a compound represented by the formula



wherein  $R^v$  represents at least one oil-solubilizing alkyl group of the type which characterizes petroleum wax, attached by one valence only to at least one aromatic nucleus  $T$ ;  $v$  represents the valence of said alkyl group  $R$  and is a small whole number from 1 to 4;  $X$  is selected from the group consisting of hydrogen and at least one metal equivalent;  $u$  is a small whole number from 1 to 4 and represents the total number of groups



attached to said alkyl group  $R^v$  through the valence  $v$ ; said compound being obtained by the reaction of one mol of phosphorus pentasulfide and substantially two mols of a compound selected from the group of compounds consisting of an alkyl-substituted hydroxyaromatic carboxylic acid and an alkyl-substituted hydroxyaromatic metal carboxylate, the alkyl substituent of said compound being at least one oil-solubilizing group of the type which characterizes petroleum wax.

9. An improved mineral oil composition comprising a mineral oil fraction having in admixture therewith a minor proportion, sufficient to stabilize said oil fraction against oxidation, of an intimate mixture of oil-soluble alkyl-substituted aromatic compounds obtained by the reaction of one mol of phosphorus pentasulfide and substantially two mols of a compound selected from the group consisting of an alkyl-substituted hydroxyaromatic carboxylic acid and an alkyl-substituted hydroxyaromatic metal carboxylate, and mono- and poly-sulfides of said carboxylic acid and of said metal carboxylate, said oil-soluble alkyl-substituted aromatic compounds of reaction being characterized by the presence of a thiophosphate ester group ( $-OPOS$ ), of a group selected from the group consisting of a thiolic acid group and a metal thiolate group ( $-COSX$ ) wherein  $X$  is selected from the group consisting of hydrogen and at least one metal equivalent, and of at least one oil-solubilizing alkyl substituent, and said compounds differing from each other with respect to the nature of said alkyl substituents which are comprised essentially of aliphatic hydrocarbon groups corresponding substantially to the different aliphatic hydrocarbons contained in paraffin wax.

10. An improved mineral oil composition comprising a mineral oil fraction having in admixture therewith a minor proportion, sufficient to stabilize said oil fraction against oxidation, of an intimate mixture of oil-soluble alkyl-substituted aromatic compounds obtained by the reaction of one mol of phosphorus pentasulfide and substantially two mols of an alkyl-substituted hydroxyaromatic carboxylic acid, said oil-soluble alkyl-substituted compounds of reaction being characterized by the presence of a thiophosphate ester group ( $-OPOS$ ), of a thiolic acid group

( $-COSH$ ), and of at least one oil-solubilizing alkyl-substituent, and said compounds differing from each other with respect to the nature of said alkyl substituents which are comprised essentially of aliphatic hydrocarbon groups corresponding substantially to the different aliphatic hydrocarbons contained in paraffin wax.

11. An improved mineral oil composition comprising a mineral oil fraction having in admixture therewith a minor proportion, sufficient to stabilize said oil fraction against oxidation, of an intimate mixture of oil-soluble alkyl-substituted aromatic compounds obtained by the reaction of one mol of phosphorus pentasulfide and substantially two mols of an alkyl-substituted hydroxyaromatic metal carboxylate, said oil-soluble alkyl-substituted aromatic compounds of reaction being characterized by the presence of a thiophosphate ester group ( $-OPOS$ ), of a metal thiolate group ( $-COSM$ ), and of at least one oil-solubilizing alkyl substituent, and said compounds differing from each other with respect to the nature of said alkyl substituents which are comprised essentially of aliphatic hydrocarbon groups corresponding substantially to the different aliphatic hydrocarbons contained in paraffin wax.

12. An improved mineral oil composition comprising a mineral oil fraction having in admixture therewith a minor proportion, sufficient to stabilize said oil fraction against oxidation, of an intimate mixture of oil-soluble alkyl-substituted aromatic compounds obtained by the reaction of one mol of phosphorus pentasulfide and substantially two mols of a disulfide of an alkyl-substituted hydroxyaromatic carboxylic acid, said oil-soluble alkyl-substituted aromatic compounds of reaction being characterized by the presence of a thiophosphate ester group ( $-OPOS$ ), of a thiolic acid group ( $-COSH$ ), and of at least one oil-solubilizing alkyl substituent, and said compounds differing from each other with respect to the nature of said alkyl substituents which are comprised essentially of aliphatic hydrocarbon groups corresponding substantially to the different aliphatic hydrocarbons contained in paraffin wax.

13. An improved mineral oil composition comprising a mineral oil fraction having in admixture therewith a minor proportion, sufficient to stabilize said oil fraction against oxidation, of a thiophosphate ester-thiolic acid of wax-phenol carboxylic acid disulfide.

14. An improved mineral oil composition comprising a mineral oil fraction having in admixture therewith a minor proportion, sufficient to stabilize said oil fraction against oxidation, of a thiophosphate ester-barium thiolate of wax-phenol carboxylic acid.

15. An improved mineral oil composition comprising a mineral oil fraction having in admixture therewith a minor proportion, sufficient to stabilize said oil fraction against oxidation, of a thiophosphate ester-barium thiolate of diamyl phenol carboxylic acid.

JOHN J. GIAMMARIA.  
ORLAND M. REIFF.